

## UNITED STATES PATENT OFFICE.

CHARLES J. RATH, OF ALLIANCE, OHIO, ASSIGNOR TO NON-CORROSIVE METAL CO., OF OKLAHOMA CITY, OKLAHOMA, A CORPORATION OF OKLAHOMA.

## ALLOY AND METHOD FOR PRODUCING SAME.

No Drawing.

Application filed April 12, 1923. Serial No. 631,691.

*To all whom it may concern:*

Be it known that I, CHARLES J. RATH, a citizen of the United States, residing at Alliance, in the county of Stark and State 3 of Ohio, have invented new and useful Improvements in Alloys and Methods for Producing Same, of which the following is a specification.

This invention relates to alloys and to 10 methods of producing the same.

It is an object of this invention to provide a copper-nickel alloy capable of withstanding high temperatures and of resisting oxidation. Moreover, the invention seeks to 15 afford a metal which is characterized by a pronounced brilliancy, and durability, and which, by reason of its ductile character, may readily be forged, cast or otherwise worked.

20 Another feature of the invention has to do with the method by which the metal is produced, it being an object to afford a simple and commercially practicable process.

The metal of the best grade, such as is 25 suitable for rolling includes copper, nickel and manganese in substantially the following percentages:

Per cent.

|           |    |
|-----------|----|
| Copper    | 78 |
| Nickel    | 21 |
| Manganese | 1  |

In the manufacture of castings, phosphor tin is included and the percentages are varied somewhat as follows:

Per cent.

|              |    |
|--------------|----|
| Copper       | 50 |
| Nickel       | 48 |
| Manganese    | 1  |
| Phosphor tin | 1  |

For the cheaper grades of metal, such as 40 used in the manufacture of vessels, table ware and the like, zinc may be substituted for the phosphor tin and manganese and the elements are incorporated in substantially the following percentages:

Per cent.

|        |          |
|--------|----------|
| Copper | 50 to 65 |
| Nickel | 15 to 18 |
| Zinc   | 20 to 35 |

In producing the metal, charcoal or other 50 suitable carbonaceous material is placed in the bottom of a crucible. The charcoal, preferably, should not be granulated or pulverized, but particles about the size of a walnut are suitable. Particles of this size

will pack sufficiently tight, and due to its 55 porosity the charcoal will absorb any traces of sulphur or other chemical impurities.

Above the charcoal is placed a flux comprising in substantially equal parts, common salt, dried or burned borax and slaked 60 lime. Upon the flux and charcoal are placed the copper and nickel, which are heated to substantially fusing state.

The borax in the flux acts as a deoxidizing agent, and shields the molten metal 65 from the atmosphere and the gases of combustion. The lime absorbs any sulphur which may be given off or is contained in the gases of combustion, and by forming a coating on the wall of the crucible, prevents the other materials from penetrating 70 the same. The salt serves to reduce any copper oxide which may be formed during the melting and acts as a general cleaner for the molten alloy in causing the metal to 75 flow freely while it is being poured.

After the metals have been fused, they are covered with flux, over which is preferably placed a layer of charcoal in order 80 to prevent the gases of combustion from coming into contact with the metal during the melting operation. When the metals are sufficiently hot for pouring, which ordinarily will be after they are heated to approximately 2400 degrees F., the manganese 85 may be added, together with the magnesium and either phosphor tin or zinc.

Subsequently the top covering of charcoal and flux is removed to permit the pouring 90 of the metal.

## I claim:

1. An alloy consisting of a substantial amount of copper, not less than approximately 50%, a substantial amount of nickel, not less than approximately 15%, and a 95 small percentage of manganese.

2. An alloy consisting of the following in substantially the percentages specified: 50% copper, 48% nickel, 1% manganese and 1% phosphorus and tin.

3. A method of producing an alloy, which consists in placing upon the bottom of a crucible a suitable carbonaceous material with a flux, covering the flux and carbonaceous material with copper and nickel, heating the metals to a fusing point, covering the materials with flux and carbonaceous material, heating the metals to a 100 105

molten state, and subsequently removing the covering of carbonaceous material and flux to permit pouring of the metal.

4. The method specified in claim 3, in 5 which the flux employed comprises in substantially equal parts, common salt, borax and slaked lime.

5. A method of producing an alloy, which 10 consists in placing upon the bottom of a crucible a suitable carbonaceous material with a flux, covering the flux and carbonaceous material with copper and nickel, heating the metals to a fusing point, covering the materials with flux and carbonaceous 15 material, heating the metals to a molten state, incorporating manganese in the molten metal, and subsequently removing the covering of carbonaceous material and flux to permit pouring of the metal.

20 6. A method of producing an alloy, which consists in placing upon the bottom of a crucible a suitable carbonaceous material with a flux, covering the flux and carbonaceous material with copper and nickel, heating the metals to a fusing point, covering the materials with flux and carbonaceous 25 material, heating the metals to a molten state, incorporating manganese and phosphor

tin in the molten metal, and subsequently removing the covering of carbonaceous material and flux to permit pouring of the metal.

7. A method of producing an alloy, which 30 consists in placing upon the bottom of a crucible a suitable carbonaceous material 35 with a flux, covering the flux and carbonaceous material with copper and nickel, heating the metals to a fusing point, covering the materials with flux and carbonaceous material, heating the metals to a molten state, incorporating manganese, magnesium and phosphor tin in the molten metal, and subsequently removing the covering of carbonaceous material and flux to permit pouring 40 of the metal.

8. An alloy consisting of a substantial 45 amount of copper, not less than approximately 50%, a substantial amount of nickel, not less than approximately 15%, a comparatively small percentage of manganese, 50 and a percentage of tin and phosphorus substantially the same as the percentage of manganese.

In testimony whereof I have hereunto set my hand.

CHARLES J. RATH.